

# UNITED STATES PATENT OFFICE.

ZENSHIRO SUZUKI, OF LOS ANGELES, CALIFORNIA.

## PROCESS FOR THE PRODUCTION OF A DYESTUFF.

1,244,796.

Specification of Letters Patent. Patented Oct. 30, 1917.

No Drawing.

Application filed October 30, 1916. Serial No. 128,644.

To all whom it may concern:

Be it known that I, ZENSHIRO SUZUKI, a subject of the Emperor of Japan, residing at Los Angeles, in the county of Los Angeles and State of California, have invented a new and useful Process for the Production of a Dyestuff, of which the following is a specification.

My invention relates to the process of the production of a dye-stuff, the main object of the invention being to provide an inexpensive process of producing a sulfur-containing dye-stuff of a dark brown color, utilizing tobacco stems, which were left as waste formerly.

In carrying out my invention I first take tobacco stems, add suitable caustic alkali to the tobacco stems, and then boil said tobacco stems and caustic alkali together until the tobacco stems is dissolved.

In order to sulfurize said dissolved substance I add a quantity of sodium sulfid and sulfur, and continue to boil, stirring up carefully, until my new sulfid dye-stuff is produced.

The following is an illustration as to the carrying out of my invention:

I preferably take one pound of tobacco stems, ten ounces of caustic soda and  $\frac{1}{2}$  gallon of water, and boil together until a thick alkali liquid of an organic chemical nature is obtained.

To said alkali liquid I next add one pound of sodium sulfid and ten ounces of sulfur.

and continue boiling, stirring the mixture well all the while. Then at first a vapor arises, sulfureted hydrogen gas following it, and there is left a strong viscous lump or mass in the boiler. I continue to heat said substance, and will by this reduce the mass to a dry mass, which may be reduced to a powder and is a new and useful sulfur-containing dye-stuff.

In order to get a different degree of color I may add at the beginning of the process to said tobacco stems, either rice straw or wheat straw; and then through the same steps as described above such desired purpose will be accomplished.

The dye-stuff I have obtained is to be used for dyeing cotton yarns and cotton goods as ordinary sulfid dye-stuff is used.

What I claim and desire to secure by Letters Patent of the United States is:

1. The method of making a sulfur-containing dye consisting essentially in heating tobacco stems with water and caustic alkali, adding sulfur and sodium sulfid and continuing the heating until sulfureted hydrogen has been evolved.

2. The method of making a sulfur-containing dye consisting essentially in heating tobacco stems with water and caustic alkali, adding sulfur and sodium sulfid and continuing the heating until a dry mass is obtained.

ZENSHIRO SUZUKI.